

# United States Patent [19]

Wasley et al.

[11] 3,932,124

[45] Jan. 13, 1976

[54] **PROCESS FOR SETTING TEXTILES**

[75] Inventors: **William L. Wasley**, Pacific Grove; **Allen G. Pittman**, El Cerrito, both of Calif.

[73] Assignee: **The United States of America as represented by the Secretary of Agriculture**, Washington, D.C.

[22] Filed: **Sept. 9, 1974**

[21] Appl. No.: **504,643**

## Related U.S. Application Data

[63] Continuation-in-part of Ser. No. 436,264, Jan. 24, 1974.

[52] U.S. Cl. .... **8/127.5; 8/128 R; 8/130.1; 428/270**

[51] Int. Cl.<sup>2</sup> .... **D06M 3/02**

[58] Field of Search .... **8/127.5, 128 R, 130.1; 117/141; 428/270**

## [56] References Cited

### UNITED STATES PATENTS

2,400,377 5/1946 Speakman ..... 8/128 R

|           |         |                 |         |
|-----------|---------|-----------------|---------|
| 2,740,727 | 4/1956  | Littleton ..... | 117/141 |
| 3,102,774 | 9/1963  | Koenig .....    | 117/141 |
| 3,514,249 | 5/1970  | Bullington..... | 8/130.1 |
| 3,617,204 | 11/1971 | Pirie.....      | 8/130.1 |

## OTHER PUBLICATIONS

Chem. Abst., 49: 5866, 1955.

Primary Examiner—Theodore Morris  
Attorney, Agent, or Firm—M. Howard Silverstein;  
William Takacs; Max D. Hensley

## [57] ABSTRACT

Wool or other protein textiles are provided with a durable set by arranging them in a predetermined pattern, and while constrained in such pattern contacting them with a hydroxylic liquid—i.e., ethylene glycol, propylene glycol, glycidol, glycerol, or diethylene glycol—under controlled conditions of time and temperature.

12 Claims, No Drawings

## PROCESS FOR SETTING TEXTILES

This is a continuation-in-part of our co-pending application, Ser. No. 436,264, filed Jan. 24, 1974.

## DESCRIPTION OF THE INVENTION

The invention relates to and has among its objects the provision of novel procedures for setting wool or other protein textile, that is, for imparting to the textile durable creases, pleats, folds, or other structural arrangements as may be desired by the operator. Further objects of the invention will be evident from the following description wherein parts and percentages are by weight unless otherwise specified.

In the following description the application of the invention to wool is emphasized. This is by way of example, not limitation. In its broad compass the invention may be utilized for the setting of all kinds of proteinous textiles.

Wool is a very useful fiber and is employed in the fabrication of numerous articles, particularly weaving apparel. It is well-known that garments of all types need to be provided with some sort of fabric arrangement, for example, pleats, creases, folds, etc. Such arrangements are conventionally produced by ironing the garment while constrained in the desired pattern. However, these arrangements are but temporary and when the garment is subjected to wear or is exposed to humid conditions, the creases, pleats, etc. disappear, leaving the garment in a shapeless condition. Procedures are also known wherein chemicals such as sodium bisulphite or ethanolamine are applied to the textile which is then steamed while held in the desired pattern. Although such procedures provide better results than pressing alone, the setting is not durable so that when the garment is laundered, the creases, pleats, or other arrangements are largely dissipated. Another disadvantage resulting from setting with bisulphites and/or amines is that they impart disagreeable odors to the product and these odors are intensified when the product is subjected to moisture and warmth, for example, when the treated garments are worn in warm or humid places.

The present invention provides a means for obviating the problems outlined above. A primary advantage is that the fabric arrangements provided by the invention are durable, that is, they are essentially permanent in practical consideration. The treated textiles may be subjected to soaking in cold or even boiling water without loss of the structure imparted thereto. Garments treated in accordance with the invention may be worn in the rain or subjected to other humid conditions without loss of pleats, creases, etc. The treated textiles may be subjected to dry cleaning or even washing in conventional aqueous soap or detergent formulations with little or no detriment to the creases, pleats, or other arrangements as may be present.

A most significant advantage of the invention is that the durable arrangements are established without impairing the desirable properties of the textile. That is to say, such properties as color, hand, elasticity, porosity, resilience, strength, wear-resistance, etc. are not harmed. For example, textiles treated in accordance with the invention exhibit essentially the same hand as the original fabric. This is in utter contrast to prior processes which depend for their effectiveness on the application of shellac, gums, starches, resins, or other high-molecular weight materials. In those cases there is

a substantial stiffening of the material so that the original hand of the fabric is impaired.

Another advantage of the invention is that no unpleasant odor is imparted to the textile. Other items to be mentioned are that the agents used in the process are inexpensive, commercially-available, and non-corrosive. Moreover, the process is outstanding in its utter simplicity and efficiency.

A further advantage is that the invention has extensive utility and can be applied to textiles which consist entirely of protein fibers (e.g., wool; mohair; silk; camel or other animal hair; regenerated protein fibers such as those prepared from casein, soybeans, peanut protein, zein, gluten, egg albumin, collagen, or keratins such as feathers, animal hoof or horn, etc.) and to textiles which contain at least 25% of protein fibers, typically blends of wool or other protein fibers with other natural or synthetic fibers such as cotton, linen, hemp, jute, ramie, sisal, cellulose acetate, cellulose acetate-butyrate, saponified acetate rayons, viscose rayons, cuprammonium rayons, ethyl cellulose, polyurethane, polyacrylonitrile, polyesters such as polyethylene terephthalate, and the like. The term "proteinous textile" is used herein as inclusive of all-protein textiles and blends which contain at least 25% protein fibers. The textile material to which the invention is applied may be in the form of bulk fibers, yarns, sliver, roving, top, webbing, card, tape, or woven or knitted fabrics, garments, or garment parts.

As noted above, an advantage of the invention is that it does not cause any damage to the intrinsic properties of the textile. Thus it does not decrease such vital attributes as hand and abrasion resistance. As a consequence, the treated textiles are suitable for all conventional uses of textiles as in fabrication of suits, shirts, skirts, and garments of all kinds. It is further to be noted that the process of the invention is outstanding in its simplicity and can be carried out with conventional equipment to be found in any textile-treating plant.

Another advantage of the invention is that the herein-described procedure may be used in conjunction with conventional textile-finishing techniques—such as dyeing, shrinkproofing, setting, and the like—without interfering with the results attained by such finishing treatments. In fact, enhanced results are often attained as explained below.

An additional advantage of the invention is that the treated textiles are more easily dyed in that they have enhanced dye-receptivity. Moreover, the treated fibers can be dyed by conventional dyes and the imparted colors are essentially permanent and not removed by laundering.

In our copending application (Ser. No. 436,234) referred to above, we have described a process for increasing the stretchability of wool textiles by contacting the textile with a hydroxylic liquid under controlled conditions of time and temperature. The instant process is related to that of 436,234 in that the same hydroxylic liquids are used (ethylene glycol, propylene glycol, glycidol, glycerol, or diethylene glycol) and they are applied under the same conditions of time and temperature. However, the instant process differs from 436,234 in the following respect:

In a practice of the present invention, the textile is first arranged in a desired pattern. This arrangement may involve laying the material flat, or folding the material, or arranging it in desired creases or pleats, or shaping it on suitable mandrels or dies. For example, in

applying the process to garments, these articles are laid on a flat surface with the desired areas folded over, creased, or otherwise arranged as conventional in preparing garments for pressing. Where more complex configurations are involved the textile may be compressed between dies having the desired shape. For example, ribbed effects may be obtained by constraining the fabric between dies having corrugated surfaces; pleated effects may be obtained by constraining the fabric between dies having mating V-shaped projections. Yarns may be crimped by compressing between corrugated surfaces, by knitting them into fabrics, by twisting them about themselves or about a rod, or by forcing them into a stuffing box. Further extensions of these principles will be obvious to those versed in the textile art.

In any event, the textile while constrained in the arranged pattern is contacted, under particular conditions, with any one of certain hydroxylic liquids, namely, ethylene glycol, glycidol, propylene glycol, glycerol, or diethylene glycol. The conditions of the treatment have been found to be critical and the desired results are attained by a correlation of time and temperature for each particular liquid.

In the case of treatment with ethylene glycol or glycidol, the temperature of treatment may range from 120° to 180° C., and the time of treatment is governed by the equation -

$$T = 175 \pm 10 - 16.7 \log t \quad (I)$$

wherein T is the temperature in degrees Centigrade, and t is the time in seconds.

By operating within the limits of Equation I, the desired results of the invention are realized. Most importantly, the desired durable set is imparted to the textile. Moreover, by operating under such conditions, there is little or no discoloration of the textile, it suffers little or no loss of tensile strength, and it retains its original hand. Typical examples of operating conditions within the limits of Equation I are given below by way of illustration:

| Temp., °C | Time, sec.                    |
|-----------|-------------------------------|
| 140       | 31 to 495, preferably 260     |
| 150       | 8 to 124, preferably 30 to 60 |
| 160       | 2 to 31, preferably 16        |

Our researches have shown that both under- and over-treatment are undesirable since they do not attain the results of the invention. For example, if the process is carried out at a selected temperature within the specified range but for a time less than that calculable from Equation I, a useful set is not attained. Any degree of set which may be obtained is not durable, and disappears when the textile is exposed to water. Moreover, if the time is increased above that calculable from the equation, inferior results are also obtained. These include discoloration, weakening of the fibers, and deterioration of hand so that in aggravated cases the product is rubbery when wet but boardy and brittle when dry.

In the case of treatment with propylene glycol, glycerol, or diethylene glycol, the temperature may range from 140° to 180° C., and the time of treatment is governed by the equation -

$$T = 188 \pm 8 - 16.7 \log t \quad (II)$$

wherein T is the temperature in degrees Centigrade, and t is the time in seconds.

In the same way as explained above, if the treatment is carried out at times or temperatures below or above those governed by Equation II, inferior results are obtained. Typical examples of operating conditions within the limits of Equation II are given below by way of illustration:

|    | Temp., °C | Time, sec.                |
|----|-----------|---------------------------|
| 10 | 150       | 63 to 562, preferably 300 |
|    | 160       | 16 to 142, preferably 130 |
|    | 170       | 4 to 34, preferably 20    |

15 Contact between the hydroxylic liquid and the constrained textile may be accomplished in various ways. The simplest and preferred method is to immerse the constrained textile in a heated bath of the hydroxylic liquid. After the period of time necessary to produce the benefits of the invention, the textile is removed 20 from the bath, and while still under constraint, is immediately cooled to below 100° C.—usually to room temperature—in order to quench (arrest) the reaction.

In an alternative procedure the treatment with the hydrolytic liquid is carried out as follows: The constrained textile is impregnated with the selected hydrolytic liquid and passed through an oven or other heating chamber wherein it is brought to the desired temperature and held thereat for the appropriate time. The treated textile is then removed from the oven and immediately cooled while still under constraint.

Other methods for effecting contact between the hydroxylic liquid and the constrained textile will be obvious to those skilled in the art. It should be noted that the process of the invention is readily adapted to continuous or batch procedures, whichever is desired.

35 The cooling operation can be carried out in various ways. For example, the treated textile while still constrained can be immersed in cold (tap) water, or in water which is cooled by addition of ice or by the use of refrigerated coils, or the like. Alternatively, the constrained textile can be cooled by subjecting it to a blast of cold air or a spray of cold water or carbon dioxide snow. Another plan is to cool the constrained textile by contact with a chilled non-aqueous inert liquid such as trichloroethane, perchloroethane, hexane, or a fluorocarbon such as difluorodichloromethane. After cooling, the textile need no longer be held under constraint; the setting has been accomplished.

50 After cooling, the textile is treated to remove any hydroxylic liquid which remains on it. Since the hydroxylic liquids are soluble in water, this is most readily accomplished by washing with water. Alternatively, the residual hydroxylic liquid is removed by washing with a non-aqueous, volatile, inert solvent such as methanol, ethanol, trichloroethane, perchloroethylene, and the like.

55 After removal of residual hydroxylic liquid, the treated textile is dried in conventional manner and is then ready for use or sale.

In an alternative modification of the invention, a minor amount (about 0.01 to 0.5%) of an acid is added to the hydroxylic liquid prior to contact with the textile, whereby to minimize possibility of discoloration of the textile. For this purpose one can use acids such as p-toluenesulphonic acid, benzene sulphonic acid, sulphuric acid, sulphamic acid, phosphoric acid, hydrochloric acid, ascorbic acid, etc. Preferably, p-toluenesulphonic acid is used in a concentration of about 0.2%.

## EXAMPLES

The invention is further demonstrated by the following examples provided by way of illustration and not limitation.

## EXAMPLE 1

A sample of mohair top was arranged in a thin layer between two stainless steel screens with mating serrated configuration which imparted crimp to the fibers. The assembly was immersed for 1 minute in ethylene glycol (at a temperature of 150° C.) which contained 0.2% p-toluene sulfonic acid. The assembly was removed from the bath and rinsed for a minute in running tap water (16 to 20° C.). The crimped fibers were removed from the assembly and were dried. The fibers retained their crimped configuration even after being placed in boiling water for 30 minutes.

## EXAMPLE 2

The procedure described in Example 1 was applied to a sample of wool top. The imparted crimp was retained although the treated sample was immersed in boiling water for 30 minutes.

## EXAMPLE 3

Very tightly-knit fabrics were made from fine crimp-free mohair yarn and from coarse, relatively crimp-free, carpet wool yarn. These knitted materials were each immersed for 60 seconds in ethylene glycol at a temperature of 150°-152° C. The treated knits were removed from the bath, were rinsed in cool tap water, and then were dried.

The treated fabrics were unraveled and the recovered yarns examined. It was found that in both cases, the yarns had acquired a high degree of crimp. For example, microscopic examination of the treated mohair yarn revealed that the individual fibers had a high degree of crimp, whereas the untreated mohair fibers were characteristically smooth and lacking in crimp. The crimped yarns could be re-knit to form fabrics having a desirable high bulk and greatly improved resiliency.

## EXAMPLE 4

Samples of wool fibers and mohair fibers were wound tightly around a glass rod (about 3/16 inch diameter). The assembly was immersed in ethylene glycol at 145° C. for a period of 75 seconds. Afterward, the assembly was removed from the bath, was rinsed with tap water, and was dried. The treated fibers were removed from the rod and they exhibited a curled configuration, which was retained even after prolonged soaking in hot water.

## EXAMPLE 5

A worsted wool fabric (4.5 oz. per sq. yd., plain weave) was constrained in a pleated configuration between two stainless steel screens having mating V-shaped conformation. The assembly was immersed for 60 seconds at a temperature of 150° C. in ethylene glycol containing 0.2% p-toluene sulfonic acid. After this treatment the assembly was immersed in cool water. The wet fabric was removed from the assembly and was dried. The sharply-pleated fabric was immersed in boiling water for 30 minutes after which time the pleats still remained.

Control: A similar piece of fabric was treated conventionally to set pleats. Thus, the fabric was constrained in the same stainless steel screen as above. The assembly was immersed for 5 min. in a boiling 2% solution of sodium bisulfite, was removed from the bath and rinsed with water, and finally was dried. The fabric was removed from the assembly and was immersed in boiling water. After 20 min. the imparted pleats were only slightly retained.

## EXAMPLE 6

A plain weave, worsted wool fabric (6.2 oz. per sq. yd.) was treated in a conventional manner to impart shrinkproofing. The conventional process entailed treating the fabric with a 2% solution of a commercial shrinkproofing agent (a polyurethane having terminal isocyanate groups) in perchloroethylene, pressing the so-treated material in a Hoffman steam press, and curing the fabric at 65% RH and 70° F. for one week.

10 A 10 in. × 14 in. swatch of the shrink-proofed fabric was constrained in both the warp and fill directions in a pin-tenter frame (device with pins on a frame useful for constraining fabrics). The assembly was immersed for 60 seconds at 150° C. in ethylene glycol containing 0.1% p-toluene sulfonic acid and then was rinsed with cool water and dried.

15 The so-treated fabric exhibited a desirable flat set, which was retained after repeated aqueous launderings.

20 The treated fabric was tested for retention of smoothness as follows. It was subjected to three washings and tumble dryings. The triple-washed fabric was then evaluated according to AATCC test method 88A-III-C, using overhead lighting procedure. In this test the fabric is rated on a scale of 1 to 5, with 5 being the most smooth and 1 being the least smooth. The treated fabric gave a rating in this test of 4.5. As a control, a sample of the same fabric was subjected to the shrinkproofing treatment alone. This fabric when tested as described had a smoothness rating of only 2.

25 30 Having thus described our invention we claim:

1. A method for imparting a stable set to a proteinous textile, which consists of -

35 a. arranging the textile in a predetermined pattern, b. while constraining it in such pattern immersing the textile in a bath consisting of ethylene glycol at a temperature in the range 120 to 180° C. and for a time governed by the limits of the equation -

$$T = 175 \pm 10 - 16.7 \log t$$

40 wherein T is the temperature in degrees Centigrade, and t is the time in seconds,

c. while still constraining the textile in the predetermined pattern immediately arresting the treatment by cooling the textile,

d. washing the textile to remove residual ethylene glycol, and drying the textile.

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 94

- d. washing the textile with water to remove residual ethylene glycol, and drying it.
4. The method of claim 3 wherein the bath consists of ethylene glycol and about 0.2% of p-toluene sulfonic acid.

5. A method for imparting a stable set to a proteinous textile, which consists of

- arranging the textile in a predetermined pattern,
- while constraining it in such pattern immersing the textile in a bath consisting of glycidol at a temperature in the range 120° to 180° C. and for a time governed by the limits of the equation -

$$T = 175 \pm 10 - 16.7 \log t$$

wherein T is the temperature in degrees Centigrade, and t is the time in seconds,

- while still constraining the textile in the predetermined pattern immediately arresting the treatment by cooling the textile,

d. washing the textile to remove residual glycidol, and drying the textile.

6. The method of claim 5 wherein the bath consists of glycidol and about 0.2% of p-toluene sulfonic acid.

7. A method for imparting a stable set to a proteinous textile, which consists of

- arranging the textile in a predetermined pattern,
- while constraining it in such pattern immersing the textile in a bath consisting of propylene glycol at a temperature in the range 140° to 180° C. and for a time governed by the limits of the equation -

$$T = 188 \pm 8 - 16.7 \log t$$

wherein T is the temperature in degrees Centigrade, and t is the time in seconds,

- while still constraining the textile in the predetermined pattern immediately arresting the treatment by cooling the textile,

d. washing the textile to remove residual propylene glycol, and drying the textile.

8. The method of claim 7 wherein the bath consists of propylene glycol and about 0.2% of p-toluene sulfonic acid.

9. A method for imparting a stable set to a proteinous textile, which consists of -

- arranging the textile in a predetermined pattern,
- while constraining it in such pattern immersing the textile in a bath consisting of glycerol at a temperature in the range 140° to 180° C. and for a time governed by the limits of the equation -

$$T = 188 \pm 8 - 16.7 \log t$$

wherein T is the temperature in degrees Centigrade, and t is the time in seconds,

- while still constraining the textile in the predetermined pattern immediately arresting the treatment by cooling the textile,

d. washing the textile to remove residual glycerol, and drying the textile.

10. The method of claim 9 wherein the bath consists of glycerol and about 0.2% of p-toluene sulfonic acid.

11. A method for imparting a stable set to a proteinous textile, which consists of

- arranging the textile in a predetermined pattern,
- while constraining it in such pattern immersing the textile in a bath consisting of diethylene glycol at a temperature in the range 140° to 180° C. and for a time governed by the limits of the equation -

$$T = 188 \pm 8 - 16.7 \log t$$

wherein T is the temperature in degrees Centigrade, and t is the time in seconds,

- while still constraining the textile in the predetermined pattern immediately arresting the treatment by cooling the textile,

d. washing the textile to remove residual diethylene glycol, and drying the textile.

12. The method of claim 11 wherein the bath consists of diethylene glycol and about 0.2% of p-toluene sulfonic acid.

\* \* \* \* \*